

Patented Feb. 14, 1928.

## UNITED STATES PATENT OFFICE.

GEORGE LANZENDORFER, OF BRAINTREE, MASSACHUSETTS, ASSIGNOR TO MARSTIN ADHESIVE COMPANY, OF BOSTON, MASSACHUSETTS, A CORPORATION OF MASSACHUSETTS.

## GLUE AND PROCESS OF PRODUCING GLUE FROM CASEIN.

No Drawing.

Application filed December 4, 1924. Serial No. 753,987.

This invention relates to improvements in processes of making glue.

Glue, as is well known, comprises an inferior grade of gelatin prepared on account of its adhesive qualities for use in the arts and industries. It is usually prepared either from the skin of an animal, particularly the corium which lies between the epidermis and inner layer of fat, or from the skin 10 scales and muscular tissue of fish.

Various means are employed for producing glue from these materials. An old process of producing glue from skins of animals consists in boiling the skins at a gentle boiling heat in soft water until the fluid attains the right consistency when it is drawn off into congealing boxes, allowed to settle, strained from impurities and finally dried.

Another method of making glue from 20 hides consists in first liming the hides to facilitate the removal of adhering flesh and fat, or treating the hides with lime, caustic soda or sulphuric acid for a like purpose, then heating the hide in water to a mild 25 boiling heat until a solution of the desired consistency is attained.

The process of producing fish glue is conducted in a similar manner. Fish skins, scales and waste muscular tissue usually are 30 employed. It is first washed, then boiled in water until the solution is of proper consistency.

These glues usually are good adhesives for wood, textile materials, paper and the like, but do not have sufficiently strong adhesive properties to adhere firmly to celluloid, metal such as aluminum and the like.

The object of the present invention is to provide a process for producing glue having 40 greater adhesive properties.

A further object of the invention is to provide a process of producing glue from substance such as casein.

Casein, a product of milk, in its commercial form, has an acid reaction due to its method of manufacture. In this condition it is not completely dispersable in water, also not in alcohol.

I have found that, for instance, equal parts 50 of casein and phenol, when the acidity is neutralized by an alkaline substance, are soluble in ethyl alcohol of 188-proof; and that four parts of casein and one part of phenol, when neutralized by an alkaline sub-

stance, are soluble in ethyl alcohol of 100-55 proof.

I have discovered that by treating a substance, such as casein, thus neutralized, with a liquid mixture comprising a suitable phenol such as cresylic acid, carbolic acid or 60 the like, and water and alcohol, in the presence of heat at a temperature of 140° F. and at atmospheric pressure, a liquid glue of strong adhesive properties will be produced.

In the performance of the process commercial casein is employed, which is obtained from milk; large quantities of such casein being imported from South America. The neutralized casein is treated with a liquid mixture comprising a phenol, water and 70 alcohol at a temperature of approximately 140° F. until a colloidal liquid of the desired consistency is obtained.

In the practical performance of the process it has been found that casein treated by 75 the above ingredients in the following proportions produces a very strong, adhesive, liquid glue. The preferred proportions are as follows:—dried casein twelve pounds, phenol four to eight pounds, (casein, as 80 commercially obtainable, varies in its property of swelling in water and hence, in order to secure a desired uniform consistency, the amount of phenol will be variable within substantially these limits), water eight 85 pounds, alcohol fourteen pounds. This mixture is gradually heated to about one hundred forty degrees temperature Fahrenheit and such heat maintained for a short time 90 when it will attain the desired consistency.

In order to overcome the acidity of the casein and also of the phenol, a mild alkali desirably is introduced into the mixture, such for example as borax, soda ash or ammonia. In the use of the ingredient in 95 the proportions above described such acidity is overcome and the alkaline nature of the glue assured by the use of approximately three pounds of borax, or one pound of soda ash, or one and one-half pounds of concentrated solution of ammonia. The term mild alkali is used as meaning such alkalis as give a low concentration of hydroxyl ions in solution as compared with "strong alkalis" such as caustic soda, which give a distinctively 100 high concentration.

It will be understood that other chemicals having like properties may be employed in

the solution for the treatment of casein or other similar substance, and that the proportions may be slightly varied as the character or conditions of the materials may vary. It will therefore be understood that the exact formula which is disclosed herein is of an illustrative character and is not restrictive and that such variations may be made as will be obvious to those skilled in the art, within 10 the meaning and scope of the following claims.

Having thus described the invention, what is claimed as new, and desired to be secured by Letters Patent, is:

- 15 1. The process of producing a casein glue which comprises treating casein with a liquid mixture comprising phenol, water, alcohol and borax in substantially the following proportions:—casein twelve pounds, phenol four to eight pounds, water eight pounds, alcohol fourteen pounds, 20 borax three pounds, in the presence of heat at approximately a

temperature of one hundred forty degrees Fahrenheit for a sufficient time to produce a liquid glue.

2. The process of producing casein glue which comprises mixing casein with a liquid mixture comprising a phenol, alcohol, water and an alkali in amount at least sufficient to neutralize the acidity of the glue in the presence of heat at approximately one hundred forty degrees Fahrenheit for a sufficient time to produce a liquid glue.

3. A liquid casein glue composition consisting of the following ingredients in substantially the following proportions: casein twelve pounds, phenol four to eight pounds, water eight pounds, alcohol fourteen pounds, and alkali in amount sufficient to neutralize the acidity of the composition.

In testimony whereof, I have signed my name to this specification.

GEORGE LANZENDORFER.